# EUROPEAN PATENT SPECIFICATION

(11) **EP 1 923 505 B1**
(45) Date of publication and mention of the grant of the patent: **23.02.2011**
(21) Application number: 07254467.9
(22) Date of filing: 15.11.2007
(51) Int. Cl.: D21H 19/64

(54) **Coated paper and paperboard**
Gestrichenes Papier und Karton
Papier revêtu et carton

(30) Priority: 20.11.2006 EP 06291798
(43) Date of publication of application: 21.05.2008
(73) Proprietor: Rohm and Haas Company, Philadelphia, PA 19106-2399 (US)
(72) Inventor: Haigh, John Robert, 06330 Roquefort-les-Pins (FR); Mukkamala, Ravi, Lansdale, PA 19446 (US)
(74) Representative: Buckley, Guy Julian

(56) References cited:
- WO-A-93/11181
- WO-A-02/059421
- US-A- 2 500 972
- US-A- 3 812 072
- US-A- 4 110 285
- US-A- 4 771 086
- US-A- 5 385 960
- DATABASE WPI Week 199333 Derwent Publications Ltd., London, GB; AN 1993-262345 XP002435488 & KR 920 008 778 B (CHEONJU PAPER CO) 9 October 1992 (1992-10-09)

## Description

This invention relates to a paper or paperboard coated with a coating having a phosphorous-containing latex and pigment.

Acrylic polymers having phosphorus-containing functional groups are known for their pigment dispersant capabilities in aqueous coating compositions (see, e.g., U.S. Pat. No. 5,385,960). WO 93/11181 discloses aqueous titanium dioxide dispersions, the dispersions comprising methacrylate phosphoric acid esters. Such polymers have also been suggested for use for making composite paper sheets with high filler levels (see, e.g., U.S. Patent No. 4,609,434). This latter patent warns, however, that such phosphorous-containing latexes can floccculate and thus be unsuitable for paper coatings. It then states that such latexes can be stabilized to a degree by copolymerizing ethylenically unsaturated carboxylic acids (such as acrylic acid) into such polymers. However, we found that copolymerizing latexes with acrylic acid does not impart sufficient viscosity stability.

This invention is a paper or paper board product comprising a paper (uncoated basis weight: 35-178 gsm) or paperboard (uncoated basis weight: 195-586 gsm) that bears (e.g., coated on one or both sides as a base coat or top coat (or any of the middle coats in case of multiple coatings applications) with) an aqueous coating composition comprising:
(a) pigment particles;
(b) particles of acrylic or vinyl polymer containing phosphate or phosphonate groups; and
(c) one or more compounds selected from a compound of formulae (I) or (II):
R1, R3, R6, R8 are independently hydrogen or alkyl groups, R2, R4, R5, R7, R9 & R10 are independently hydrogen, alkyl groups or ammonium or metal counter ions, or wherein R5 is a residue of a phosphoethyldimethacrylate that is in turn optionally polymerized with other ethylenically unsaturated monomers or dimmers; wherein each of the sums (m+n) and (q+r) is an integer from 10 to 600, and p is an integer from 1-10; and wherein each of the ratios m:n and q:r is from 0:100 to 95:5.

Some of the polymeric structures of Formula (I) or (II) are water soluble.

By "polyphosphate compound(s)," we mean linear or cyclic polyphosphate(s) at described by Cotton et al., Advanced Inorganic Chemistry, A Comprehensive Text, Interscience Publishers (1972), p. 397.

Preferred compounds polyphosphates include, e.g., the acid form, or the alkali metal or ammonium salts of pyrophosphates, tripolyphosphates, metaphosphates and polymetaphosphates [for example, (NaPO₃)ₓ, such as sodium hexametaphosphate where x = 6 or other similar structures with x is higher than 6. In a preferred embodiment of the invention, the sodium salts are used.

The weight ratio of the phosphorous-containing acrylic polymer binder to the polyphosphate compound(s) (and/or compounds of Formulae (I) or (II)) can preferably range from 1:0.001 to 1:2, more preferably from 1:0.01 to 1:0.5, and most preferably from 1:0.03 to 1:0.3.

All percentages are weight percentages, unless specified otherwise. The term "acrylic polymer" refers to a polymer comprising at least 40% monomer units derived from among the following acrylic monomers: acrylonitrile (AN); acrylamide (AM), methacrylamide, and their N-substituted derivatives; acrylic acid (AA), methacrylic acid (MAA), and itaconic acid (IA) and their esters. The terms (meth)acrylic and (meth)acrylate refer to acrylic or methacrylic, and acrylate or methacrylate, respectively. Esters of AA and MAA include, but are not limited to, methyl methacrylate (MMA), ethyl methacrylate (EMA), butyl methacrylate (BMA), ethylhexyl methacrylate (EHMA), lauryl methacrylate (LMA), hydroxyethyl methacrylate (HEMA), methyl acrylate (MA), ethyl acrylate (EA), butyl acrylate (BA), ethylhexyl acrylate (EHA) and hydroxyethyl acrylate (HEA), as well as other esters of AA or MAA, e.g., alkyl, hydroxyalkyl and aminoalkyl esters; phosphoalkyl (meth)acrylates. Phosphoalkyl (meth)acrylates include, e.g, phosphoethyl methacrylate (PEM), phosphopropyl (meth)acrylate, phosphobutyl (meth)acrylate. Derivatives of acrylamide include, e.g., methylol acrylamide (MLAM). Acrylic polymers also may contain monomer units derived from other ethylenically unsaturated monomers, e.g., styrene or substituted styrenes; other α,β-unsaturated carboxylic acids, esters and amides; vinyl esters or halides; etc. Preferably, an acrylic polymer contains at least 50% monomer residues derived from acrylic monomers, more preferably at least 60%, and most preferably at least 70%; preferably an acrylic polymer is substantially free of monomer units other than those of AA, MAA and their esters. An "acrylic-styrene copolymer" is a polymer at least 50% of whose monomer units are derived from among AA, MAA, esters of AA and MAA, and styrene monomers. Styrene monomers include styrene (Sty) and substituted styrenes, e.g., α-methylstyrene (AMS). Preferably, acrylic-styrene copolymers contain less than 20% of monomer units other than styrene or acrylic monomer units, more preferably less than 10%, and most preferably less than 5%. Preferably, a polymer in this invention is present in the form of a latex. The polymer may be unimodal or bimodal, see, e.g., U.S. Patent No. 6,818,697.

The aqueous composition of this invention comprises an acrylic polymer containing phosphate or phosphonate groups. In one embodiment of the invention, these groups are present in the form of monomer residues from phosphate- or phosphonate-containing monomers, including, e.g., phosphoalkyl (meth)acrylates such as phosphoethyl (meth)acrylate, phosphopropyl (meth)acrylate, and phosphobutyl (meth)acrylate, phosphoalkyl crotonates, phosphoalkyl maleates, phosphoalkyl fumarates, phosphodialkyl (meth)acrylates, phosphodialkyl crotonates, and allyl and vinyl phosphate. For purposes of this invention, phosphoalkyl (meth)acrylates include ethylene oxide condensates of (meth)acrylates such as H₂C=C(CH₃)COO(CH₂CH₂O)ₙP(O)(OH)₂, where n is from 1 to 50. The phosphate- or phosphonate-containing polymer may be the only acrylic polymer in the composition, or it may be blended with an acrylic polymer not containing phosphate or phosphonate groups. Preferably, the phosphate- or phosphonate-containing monomer units comprise from 0.5% to 8% of the total amount of acrylic polymer(s) on a solids basis, more preferably from 1% to 5%.

The composition used in or on the paper or paper board of this invention comprises one or more types of pigment particles. Examples of pigments include, but not limited to mineral pigments such as ground and precipitated calcium carbonate, kaolin, calcined clay, delaminated and structured clay, titanium dioxide, aluminum silicate, magnesium silicate, zinc oxide, iron oxide, magnesium carbonate, amorphous silica, zinc hydroxide, aluminum oxide, aluminum hydroxide, talc, satin white, barium sulfate and calcium sulfate, and combinations of these materials. Pigments useful in this invention can also include various polymeric plastic pigments including, but not limited to solid bead, voided, mutli-voided, binder-coated, charged, etc. and their combinations. Preferably, the composition of this invention comprises calcium carbonate. Calcium carbonate can be ground-type (GCC) or precipitated-type (PCC) of varying particle size, shape and morphologies.

Preferably, the total amount of latex polymer in the coating composition for 100 parts (dry) of total pigments combined is 1-25 parts (dry) more preferably from 3-18 parts (dry) and most preferably 5-15 parts (dry).

In one embodiment of the invention, the acrylic polymer containing phosphate or phosphonate groups has a Tg from -30°C to 60°C. Preferably, the T_{g} is from -25°C to 45°C, and most preferably from -20°C to 35°C. Tg is calculated using the Fox equation (T.G. Fox, Bull. Am. Physics Soc., vol. 1 (3), page 123 (1956)). Preferably, the weight average molecular weight (M_{w}) of the acrylic polymer is 50,000-1,500,000, more preferably at least 200,000-1,200,000, and most preferably at least 500,000-800,000.

Particle size ranges: preferably 50-500 nm, more preferably 60-350 nm and most preferably 80-300 nm. When the composition of this invention is formulated as a coating, other conventional binders known in the paper coatings art can be added in combination of the phosphorous-contaning latex. Such additional binders include (but not limited to), acrylates, styrene-acrylates, vinyl acetates, vinyl acetate-acylates, SBRs (including SB and SBAs), etc.

When the composition of this invention is formulated as a coating, other conventional coatings adjuvants typically are added, for example, tackifiers, emulsifiers, buffers, neutralizers, thickeners or rheology modifiers, humectants, wetting agents, biocides, plasticizers, antifoaming agents, optical brightening agents (OBAs), colorants, waxes, anti-oxidants, and coalescing agents. The solids content of the aqueous coating composition of the invention is from 30% to 80% by weight. The viscosity of the aqueous coating composition prior to application on the paper or paper board is preferably less than about 4000 cP, preferably more than 50 cps, as measured using a Brookfield viscometer.

The composition of this invention provides improved viscosity stability to latex formulations containing pigments and/or fillers, i.e., it reduces the change in viscosity that occurs upon equilibration or aging. The composition also may have reduced formation of masses of flocculated particles, which tend to settle out of coating compositions.

### Example 1

### Preparation of an Aqueous Dispersion of Phosphorous-Containing Polymer Particles

A monomer emulsion was prepared by combining 576 g of deionized (DI) water, 21.1 g of dodecylbenzene sulfonate surfactant (23 weight% active), 38.6 g of an ethoxylated monoalkyl sulfosuccinate surfactant (30 weight% active), 38.6 g acrylic acid, 1255.3 g butyl acrylate, 154.8 g acrylonitrile, 425 g styrene, and 57.9 g of phosphoethyl methacrylate (50% active). To a five liter, four-neck round bottom flask equipped with stirrer and condenser, and containing 664 g DI water, 12.6 g dodecylbenzene sulfonate (23%), 1.44 g sodium sulfate, and 0.4 g of 4-hydroxy TEMPO (5% active) at 87°C was charged 102.7 g of the monomer emulsion, followed by 5.9 g sodium persulfate dissolved in 32.4 g DI water, and rinsed to the flask with an additional 22.6 g DI water. After ten minutes, the remaining monomer emulsion and a solution of 5.9 g sodium persulfate and 8.6 g sodium hydroxide (50% active) in 203.4 g DI water were added separately to the flask over three hours. The temperature of the batch was maintained at 87°C during the addition. When all additions were completed, the containers were rinsed to the flask with 15.2 g DI water. Separate catalyst and activator charges consisting of 14.3 g t-butyl hydroperoxide (70%) and 8.8 g sodium bisulfite in DI water were added in three portions over 90 minutes while cooling the batch to 45°C, and a neutralizer solution consisting of 42.6 g sodium hydroxide (50%) in 253.9 g DI water was added during the same period. The batch was finished off with the addition of 8.1 g Kathon LX solution (1.4% active), and 1.17 g of Drewplus T-3200 defoamer. The aqueous polymer dispersion of Example 1 contained 49 weight % solids and had a pH of 7.6. Using this procedure, two latexes Example 1A (particle size ca. 90 nm) and Example 1B (Particle size ca. 130 nm)

### Example 2

### Preparation of an Aqueous Dispersion of Phosphorous-Containing Polymer Particles

A monomer emulsion was prepared by combining 497 g of deionized (DI) water, 19.3 g of dodecylbenzene sulfonate surfactant (23 weight% active), 17.7 g of an ethoxylated monoalkyl sulfosuccinate surfactant (30 weight% active), 44.4 g acrylic acid, 1452.9 g butyl acrylate, 88.6 g acrylonitrile, 132.9 g styrene, and 53.2 g of phosphoethyl methacrylate (50% active). To a five liter, four-neck round bottom flask equipped with stirrer and condenser, and containing 715 g DI water, 2.2 g dodecylbenzene sulfonate (23%), 2.7 g sodium sulfate, and 0.08 g of 4-hydroxy TEMPO (5% active) at 87°C was charged 69.2 g of the monomer emulsion, followed by 5.3 g ammonium persulfate dissolved in 35 g DI water. After five minutes, the remaining monomer emulsion and a solution of 5.3 g sodium persulfate in 100 g DI water, and 7.3 g sodium hydroxide (50% active) in 65 g DI water were added separately to the flask over 2.5 hours. The temperature of the batch was maintained at 86°C during the addition. When all additions were completed, the containers were rinsed to the flask with 40 g DI water. Separate catalyst and activator charges consisting of 3.8 g t-butyl hydroperoxide(70%)/ 2.7 g sodium bisulfite in 95 g DI water and 4.9 g t-butyl hydroperoxide (70%)/ 3.5 g isoascorbic acid in 110 g DI water were added, each over 30 minutes while cooling the batch to 75°C. While further cooling the batch to 45°C, charges were added in succession of 1.1 g Drewplus T-3200 defoamer, a solution of 15.4 g sodium hydroxide (50%) and 22.6 g ethoxylated monoalkyl sulfosuccinate (30%) with 48 g DI water, and 7.9 g Kathon LX solution (1.4% active)in 25 g DI water. The aqueous polymer dispersion of Example 2 contained 49.3 weight % solids and had a pH of 6.0.

### Example 3

A 5% tetra sodium pyrophosphate decahydrate solution in water was prepared by dissolving 5 grams of this material in 95 grams of water.

### Examples 4A-C

### Coating formulations and viscosity data

| | | 4A | 4B | 4C |
|---|---|---|---|---|
| Material name | | Dry Parts | Dry Parts | Dry Parts |
| Clay(20)/Calcium Carbonate (80) slurry | | 100 | 100 | 100 |
| Latex binder (example 1) | | 10 | 10 | 10 |
| RM-232 (Thickner) | | 0.2 | 0.2 | 0.21 |
| Tetra Sodium Pyrophosphate (TSPP) | | 0 | 0.5 | 1 |
| Total parts | | 110.2 | 110.7 | 111.2 |
| Coating Solids (%) | | 59 | 59 | 59 |
| Brookfield Viscosity (cP), # 3 spindle, 60 rpm | Initial | 750 | 800 | 1000 |
| | 2h | 7200 | 1275 | 1982 |

Examples 4b and 4c with tetra sodium pyrophosphate show lower viscosity build over 2h compared to 4a without tetra sodium pyrophosphate.

### Example 5

### Preparation of Sodium Hexametaphosphate Solution

A 50% sodium hexametaphosphate (Calgon-N purchased from BK Giuilini, CA, USA) solution in water was prepared by dissolving 50 grams of this material in 50 grams of water. This solution was used in the examples below, where indicated

### Examples 6A-G

### Coating Formulations and Viscosity Over Time Data

The ingredients used in the table below are Hydrocarb-90 (calcium carbonate) obtained from Omya, Inc.; SPS (clay of regular brightness) purchased from Imerys, Inc.; AF-1055 ER (hollow plastic pigment) and Primal 308 AF (styrene-acrylate binder) available as commercial products from the Rohm and Haas Company, Philadelphia, PA; Rhoplex RM-232D, a thickener (hydrophobically- modified, low foam version alkali-swellable emulsion (HASE)) also available from Rohm and Haas. These materials were used to make the following coating formulations.

| **Coatings** | | 6A | 6B | 6C | 6D | 6E | 6F | 6G |
|---|---|---|---|---|---|---|---|---|
| **Coating Ingredients** | | **Dry parts by weight (unless otherwise noted)** | | | | | | |
| **Hydrocarb 90 (calcium carbonate)** | | 70 | 70 | 70 | 70 | 70 | 100 | 100 |
| **SPS (clay)** | | 25 | 25 | 25 | 25 | 25 | | |
| **AF 1055ER** | | 5 | 5 | 5 | 5 | 5 | | |
| **Primal 308AF** | | 10 | | | | | | |
| **Latex from Example 1** | | | 10 | 10 | 10 | 10 | 10 | 10 |
| **Calgon-N solution (wt% on latex binder solids)** | | 0 | 0 | 2 | 4 | 5 | 6 | 2 |
| **Rhoplex RM 232DE** | | 0.02 | 0.02 | 0.05 | 0.02 | | | |
| | | | | | | | | |

| **Coating Solids (%)** | | **64** | **64** | **64** | **64** | **64** | **64** | **64** |
|---|---|---|---|---|---|---|---|---|
| Brookfield Viscosity (# 4 spindle, 100 rpm) | **Time (h)** | **Viscosity (cP)** | | | | | | |
| | **0** | 700 | 685 | 687 | 685 | 664 | 350 | 198 |
| | **0.25** | | 1224 | 854 | | | 580 | |
| | **0.5** | 736 | 2052 | | 907 | 878 | | 426 |
| | **0.92** | | | | | | | |
| | **2** | 766 | | 1080 | 1014 | 972 | 630 | |
| | **4** | | | | 1156 | | 780 | |
| | **5** | | | | 1276 | | | |
| | **6** | 760 | 6180 | 1534 | | 1220 | 1100 | |
| | **8** | | | | | 1350 | | |
| | **16** | | | | | | | 3830 |
| | **18.5** | | | | | | | 4160 |
| | **24** | | | 3128 | 2084 | 1664 | 1280 | |
| | **48** | 850 | | 5130 | | 1950 | | |
| | **96** | | | | 3352 | | | |

Examples 6A and 6B show that a paper coating formulation with phosphorous-containing latex shows a significant increase viscosity, and examples B-G show that this viscosity increase can be controlled by Calgon-N dispersant there by providing stable paper coating colors.

### Example 7

Coating formulations 7A-I were made (whose main ingredients are given in the table below) and coated on both sides (C2S) of a freesheet base stock (65 gsm) at the KCL (Finland) pilot coater using a jet-coater head running at 1800 m/min. The coatings 7 D-I were made from the experimental latexes 1A and 1B that were pre-mixed with 50 wt% aqueous solution of Calgon-N such that it was 3 wt% on latex solids. The applied coat weight on the sheet was 7 gsm on each side. The coated sheets were calendered on a off-line supercalender running at speed of 1500 m/min with 9 nips and at temperatures of 60-90 deg C and a pressure of 200 kN/m to a target gloss of ca. 70 as measured by the on-line gloss meter (75 deg gloss).

| **Coatings** | 7A | 7B | 7C | 7D | 7E | 7F | 7G | 7H | 7I |
|---|---|---|---|---|---|---|---|---|---|
| **Ingredients** | **Dry Parts By Weight** | | | | | | | | |
| **CaC03 Covercarb 75** | 80 | 80 | 80 | 80 | 80 | 80 | 80 | 80 | 80 |
| **Clay HG-90** | 20 | 20 | 20 | 20 | 20 | 20 | 20 | 20 | 20 |
| **Primal P-308AF** | 12 | 11 | 10 | | | | | | |
| **Exp. Latex (Example 1A+Calgon-N))** | | | | 12 | 11 | 10 | | | |
| **Exp. Latex (Example 1B+Calgon-N))** | | | | | | | 12 | 11 | 10 |
| **pH** | Ca.8.5 | | | | | | | | |
| **Solids (wt%)** | 58.5 | | | | | | | | |

Papers coated with above coatings 7A-I were tested in the lab for general optical properties (75 deg gloss using a bench top glossmeter from Technidyne (New Albany, IN)). The same papers were tested for Vandercook wet pick coating strength using a laboratory Prufbau printing station. The conditions for the wet pick coating strength tests were as the following: sheet-fed cyan ink (0.18 g), pressure, 800N; printing speed, 1.2 m/s; inking time, 30 sec; water: 10 microliter droplet. The prints are rated from 1-5 where 1 is represents the highest strength and 5 the lowest.

| **Coatings** | 7A | 7B | 7C | 7D | 7E | 7F | 7G | 7H | 71 |
|---|---|---|---|---|---|---|---|---|---|
| **Gloss (75 deg)** | 69 | 73.5 | 72.9 | 70.9 | 73.1 | 73.8 | 70.6 | 71.8 | 71.3 |
| **Wet Pick rating** | 4 | 3 | 5 | 2 | 2 | 2 | 3 | 2 | 2 |

The ratings above show that the experimental latexes with phosphate monomers incorporated impart higher coating strength compared to the regular styrene-acrylate latex.

## Claims

1. A paper or paper board product comprising a paper (uncoated basis weight: 35-178 gsm) or paperboard (uncoated basis weight: 195-586 gsm) that bears an aqueous coating composition comprising:
(a) pigment particles;
(b) particles of acrylic or vinyl polymer containing phosphate or phosphonate groups; and
(c) one or more compounds selected from a compound of formulae (I) or (II):
R1, R3, R6, R8 are independently hydrogen or alkyl groups,
R2, R4, R5, R7, R9 & R10 are independently hydrogen, alkyl groups or ammonium or metal counter ions, or wherein R5 is a residue of a phosphoethyldimethacrylate that is in turn optionally polymerized with other ethylenically unsaturated monomers or dimmers;
wherein each of the sums (m+n) and (q+r) is an integer from 10 to 600, and p is an integer from 1-10; and wherein each of the ratios m:n and q:r is from 0:100 to 95:5.

2. The paper or paper board product of claim 1 wherein the pigment particles are selected from among the group consisting of titanium dioxide, zinc oxide, clay, talc, calcium carbonate and combinations thereof.

3. The paper or paper board product of claim 1 wherein the composition comprises calcium carbonate.

4. The paper or paper board product of claim 1 wherein the acrylic polymer containing phosphate or phosphonate groups has a Tg from -30°C to 60°C.

5. The paper or paper board product of claim 4 wherein the acrylic polymer containing phosphate or phosphonate groups comprises residues of phosphoalkyl (meth)acrylate.

6. The paper or paper board product of claim 1 wherein the coating composition prior to application on the product has a viscosity of less than about 4000cP.

## Patentansprüche

1. Papier- oder Pappeprodukt, das ein Papier (unbeschichtetes Basisgewicht: 35 bis 178 g/m²) oder Pappe (unbeschichtetes Basisgewicht: 195 bis 586 g/m²) umfasst, das oder die eine wässrige Beschichtungszusammensetzung aufweist, umfassend:
(a) Pigmentteilchen,
(b) Teilchen eines Acryl- oder Vinylpolymers, enthaltend Phosphat- oder Phosphonatgruppen und
(c) eine oder mehrere Verbindung(en), die aus einer Verbindung der Formeln (I) oder (II) ausgewählt ist oder sind: R1, R3, R6, R8 sind unabhängig Wasserstoff oder Alkylgruppen,
R2, R4, R5, R7, R9 und R10 sind unabhängig Wasserstoff, Alkylgruppen oder Ammonium- oder Metallgegenionen, oder wobei R5 ein Rest eines Phosphoethyldimethacrylats ist, der wiederum gegebenenfalls mit anderen ethylenisch ungesättigten Monomeren oder Dimeren polymerisiert ist,
wobei jede der Summen (m+n) und (q+r) eine ganze Zahl von 10 bis 600 ist und p eine ganze Zahl von 1 bis 10 ist, und wobei jedes der Verhältnisse m:n und q:r 0:100 bis 95:5 ist.

2. Papier- oder Pappeprodukt nach Anspruch 1, bei dem die Pigmentteilchen aus der Gruppe, bestehend aus Titandioxid, Zinkoxid, Ton, Talk, Calciumcarbonat und Kombinationen davon, ausgewählt sind.

3. Papier- oder Pappeprodukt nach Anspruch 1, bei dem die Zusammensetzung Calciumcarbonat umfasst.

4. Papier- oder Pappeprodukt nach Anspruch 1, bei dem das Acrylpolymer, das Phosphat- oder Phosphonatgruppen enthält, eine T_{g} von -30°C bis 60°C aufweist.

5. Papier- oder Pappeprodukt nach Anspruch 4, bei dem das Acrylpolymer, das Phosphat- oder Phosphonatgruppen enthält, Phosphoalkyl(meth)acrylat-Reste umfasst.

6. Papier- oder Pappeprodukt nach Anspruch 1, bei dem die Beschichtungszusammensetzung vor dem Aufbringen auf das Produkt eine Viskosität von weniger als etwa 4000 cP aufweist.

## Revendications

1. Produit de papier ou de carton comprenant un papier (poids de base non revêtu : 35-178 g/m²) ou un carton (poids de base non revêtu : 195-586 g/m²) qui porte une composition de revêtement aqueuse comprenant :
(a) des particules de pigment ;
(b) des particules d'un polymère acrylique ou vinylique contenant des groupes phosphate ou phosphonate ; et
(c) un ou plusieurs composés choisis parmi un composé des formules (I) ou (II) :
R1, R3, R6, R8 sont indépendamment un atome d'hydrogène ou des groupes alkyle,
R2, R4, R5, R7, R9 et R10 sont indépendamment un atome d'hydrogène, des groupes alkyle ou des contre-ions ammonium ou métalliques, ou dans lesquelles R5 est un résidu d'un diméthacrylate de phosphoéthyle qui est à son tour éventuellement polymérisé avec d'autres monomères ou dimères éthyléniquement insaturés ;
dans lesquelles chacune des sommes (m+n) et (q+r) est un nombre entier de 10 à 600 et p est un nombre entier de 1-10 ; et dans lesquelles chacun des rapports m:n et q:r est compris entre 0 : 100 et 95 : 5.

2. Produit de papier ou de carton selon la revendication 1, dans lequel les particules de pigment sont choisies dans le groupe constitué de dioxyde de titane, d'oxyde de zinc, d'argile, de stéatite, de carbonate de calcium et de combinaisons de ceux-ci.

3. Produit de papier ou de carton selon la revendication 1, dans lequel la composition comprend du carbonate de calcium.

4. Produit de papier ou de carton selon la revendication 1, dans lequel le polymère acrylique contenant des groupes phosphate ou phosphonate présente une Tg de -30°C à 60°C.

5. Produit de papier ou de carton selon la revendication 4, dans lequel le polymère acrylique contenant des groupes phosphate ou phosphonate comprend des résidus de (méth)acrylate de phosphoalkyle.

6. Produit de papier ou de carton selon la revendication 1, dans lequel la composition de revêtement présente avant l'application sur le produit une viscosité inférieure à environ 4 000 cP.
